

# United States Patent Office

2,847,374

Patented Aug. 12, 1958

1

2,847,374

## METAL PROCESSING

Hugh G. Webster and Robert H. Shoemaker, Detroit, Mich., assignors to Kolene Corporation, Detroit, Mich.

No Drawing. Application June 12, 1956  
Serial No. 590,840

8 Claims. (Cl. 204—145)

This invention relates to improved heat treating and electrolytic cleaning of metals to remove surface impurities such as oxides and scales usually associated therewith by placing the metal work piece in a molten salt type of bath and subjecting same to electrolysis in which the metal work piece is alternately electrolyzed with direct current, first as a cathode and then as an anode.

The metal work piece is usually of ferrous metal, but it may be of non-ferrous metal. An outstanding bath for cleaning of metal of this character is known in the art, as the K-4 bath, and is particularly described in prior Patent No. 2,468,006. That bath preferably comprises 75—90% of caustic, either sodium or potassium hydroxide and small proportions, such as 7—13% of sodium chloride and 0.5—5% of sodium aluminate, all proportions by weight. When the metal work piece contains sand or silica inclusions in the surface usually resulting from casting, the bath may further contain 2—6% of alkali metal fluoride. While that bath has had great commercial success in the cleaning of metal as described in that patent, for purposes of the present invention the electrolytic cleaning bath may be further varied to contain minor contents, 0.5—15% of alkali metal borate, 1—15% of alkali metal fluoroborate, 1—10% of alkali metal cyanide, 1—15% of alkali metal fluo-silicate or 1—10% of alkali metal silicate.

It is usually found desirable to preheat metal, particularly ferrous metal at a temperature ranging from 1100 to 1350° F., usually around 1200° F., for purposes of stress-relieving the metal. That primary heat treatment for stress-relieving according to the present invention, is performed in a molten salt bath, primarily because it is possible by that molten salt bath heat treatment to secure optimum heat transfer to all parts of the metal and because it is possible in such bath to obtain an exact temperature control at which the metal is heated to obtain optimum stress relief.

The electrolytic treatment in a salt bath, as described above, gives by far the best cleaning and descaling of the metal surface. The cleaning operation by electrolysis in such molten salt bath, however, is usually at a considerably lower temperature possibly applied in the range from 600 to 1000° F., but preferably from 850 to 900° F. Accordingly, it is not practically possible to simultaneously use the same electrolytic cleaning bath for heating the metal to stress relieve it, before application of electrolysis to clean it.

Where metal is cleaned in certain known molten salt baths whose composition is fundamentally different from that used for electrolytic cleaning, there may be an attack upon the metal oxides and scale on the metal, without electrolysis, particularly, when the bath contains an oxidizing agent like a nitrate salt. Such bath is inferior to an electrolytic bath as described above, for cleaning the metal, but more important, such bath will both corrode the bath apparatus at the higher stress-relieving temperature and often convert the oxide and scale on the

2

metal to a form rendering them even more difficult to remove by electrolysis in an electrolytic cleaning bath of the character mentioned above. Moreover, if such varied composition stress-relieving bath were used, it would necessitate, after removal of the metal from the stress-relieving bath, cooling the metal sufficient to wash the adhered molten or solidified salts from the surface and drying of the metal before immersion in the electrolytic cleaning bath. On the other hand, if the metal were taken from the stress relieving bath, cooled with the molten salt thereon and passed directly into the electrolytic cleaning bath, the cleaning bath would soon become so contaminated with undesirable salt components carried over from the stress-relieving bath that the electrolytic cleaning operation would become considerably inferior and, in a short time, the electrolytic cleaning bath would be rendered useless by the accumulation of such contaminating materials.

It is a primary object of the present invention to provide a stress-relieving bath which, without electrolysis in the stress-relieving heat treatment, does not adversely affect the adherent surface impurities upon the metal such as oxides and scale.

It is a further object to form such bath of molten salt materials capable both of functioning satisfactorily for stress-relief and which, upon subsequent transfer from the stress-relieving bath without removal of molten salt thereon to the electrolytic cleaning bath, will not substantially contaminate the cleaning bath or in any wise interfere with the efficient electrolytic cleaning operation.

This invention is based in part upon the discovery that molten salt baths of the type described above, which are useful for cleaning of metals, particularly ferrous metal, electrolytically, will not, in the absence of applied electrolysis to such molten salts, adversely affect the oxide or scale upon the metal, whereby such molten salts, useful for electrolytic cleaning, are also eminently suitable materials for a stress-relieving bath. Furthermore, when metal is stress-relieved in such bath materials by subjecting to a temperature in the above mentioned stress-relieving range, upon removal from such bath after heat treating, the metal does not need to have the adherent molten salts removed, since they may be of the same character as the bath used for electrolytic cleaning. Thus, the metal, after heating for stress-relief and removal from that molten salt bath coated with adherent molten salts, may be directly placed in another bath of substantially the same molten salt material at a lower temperature and electrolyzed to effect the cleaning thereof in a manner known in the art, for instance, as described in patent above identified.

It will be appreciated that using the same bath materials for both baths, the first bath for stress relieving without electrolysis and the second bath subsequently for electrolyzing to clean the metal, the transfer of molten salt from one bath to the other does not tend to adversely vary the composition of the cleaning bath. Moreover, by use of the electrolytic type of bath for stress-relieving, the oxide and scale coating upon the metal is not affected in a manner whereby the subsequent electrolysis is performed less advantageously than in usual electrolytic cleaning with baths of this character.

In another aspect of this invention, we have found that subjecting a bath of this type to the extremely high temperature necessary for stress-relieving for long periods of time without electrolysis, tends to make the bath somewhat corrosive to the heating apparatus, which, and over long periods of time, may be severe upon large tanks comprising the stress relieving apparatus.

It is found however, that the tendency to corrode the stress-relieving apparatus may be overcome by passing

into the molten salt stress-relieving bath of the character described, water vapors, i. e., steam, preheated to a temperature that will not substantially affect the temperature of the bath. Alternatively, it is found that addition of certain hydrated salts which will decompose and release water vapor at the high temperatures involved will overcome the corrosive effect upon the stress-relieving apparatus.

That hydrated salt should be of an alkali or alkali earth metal. For instance, it may be one of the salts normally forming the bath of the type above mentioned, which contains water of crystallization, for instance, a hydrated alkali-forming metal borate or a hydrated caustic alkali, but is preferably a hydrated alkali earth salt which does not lose its water of hydration until subjected to high temperatures to melt it or dissolve it in the molten salts of the bath. For this purpose alkali earth metal hydroxides which are hydrated and tend to bond the water of hydration without release until relatively high temperatures are reached, may be used.

The various alkali earth metal hydroxides such as barium, calcium or strontium hydroxides containing water of crystallization may be used; and of this group, barium hydroxide is preferred because it does not appear to adversely affect the fluidity as well as other desirable properties of the bath, and particularly, as it accumulates in the subsequent cleaning bath does not adversely affect the operation thereof in contrast to other diluents carried over from the stress-relieving bath which are often objectionable.

Accordingly, it is a further object of this invention to impart a water vapor content to the stress-relieving bath to inhibit corrosion either by way of addition of steam directly to the bath at about the temperature of the bath, or by addition of hydrated salts which release water vapor in the molten salt bath. As additive salts, preferably we use hydrated salts to supply water vapor to the stress-relieving bath of the same kind as appear in the electrolytic cleaning bath, except that alkali earth metal hydrate, preferably barium hydrate, may be used in the stress-relieving bath in the form of their hydrates for supply of water vapor thereto.

Where an alkali earth metal hydrate is added to the stress-relieving bath it will be present in proportion of about 1 to 15% for humidification thereof. Where the humidification is effected by passing steam into the stress-relieving bath, it may be added as a continuous supply of steam bubbled into the bath at the rate of about 1 to 100 lbs. per hour, per 1000 lbs. or molten bath salts; or the bath may be treated with steam periodically by supplying 1 to 5 lbs. of steam passed into the bath over a period of 1/2 to 2 hours every 5 to 24 hours, as a series of intermittent applications.

It will be understood that the treatment of the stress-relieving bath with steam or addition thereto of salts capable of releasing water of crystallization is for the purpose of offsetting the corrosive effects of the stress-relieving salts upon the apparatus containing the molten salt stress-relieving bath. Where that specific function to prevent corrosion is not needed for the specific apparatus, that type of treatment may be omitted.

The following examples illustrate the practice of this invention:

#### Example I

Two baths, both having the same composition, consisting of 85% sodium hydroxide, 10% sodium chloride, 4% sodium fluoride and 1% sodium aluminate, by weight, are made up in separate tanks by heating the composition above the melting point thereof. The tank for cleaning the metal may have the same construction as shown in prior application, Ser. No. 239,934, now Patent No. 2,732,339. The tank for stress-relieving may be of the same construction, except that electrodes are omitted. The stress-relieving tank is heated to a temperature of 1200° F. The electrolytic cleaning bath

is heated to 875° F. Gray iron castings are first placed in the stress-relieving tank and held therein for one hour, thereby being heated at 1200° F., in the molten salt composition. The castings are then removed from the stress-relieving tank and transferred to the cleaning tank wherein they are made first a cathode and current is passed therethrough for a period of 20 minutes at a volatge drop of 2 1/2 to 6 volts, using 1000 amperes' current for each 4000 lbs. of bath composition. Thereafter, the current is reversed to make the castings an anode for a period of about 10 minutes and finally reversed again whereby the work pieces are then withdrawn from the bath and the molten salt washed off with water; they are found to be clean as well as stress-relieved.

While in the foregoing example the work is first cathodic, then anodic, and finally cathodic again, after which the work is withdrawn from the bath, there are other and many instances where the work is cathodic only, without any reversal of current.

#### Example II

The procedure for stress-relieving and cleaning metal as set forth in Example I is repeated, except that a molten salt bath and stress-relieving composition, the same composition for both baths, is substituted as follows: 81% of sodium hydroxide, 5% sodium tetraborate decahydrate (borax), 4% sodium fluoride and 10% sodium chloride. It was found that the bath substance of this example showed no tendency to corrode the stress-relieving bath over a period of 5 days of continuous use, whereas that of Example I showed signs of incipient corrosion of the tank walls of the stress-relieving bath. However, upon continued use of the bath of this example for 2 weeks, the stress-relieving bath too began to show signs of corrosion thereby indicating that the capacity to evolve water vapor for protection of the tank is exhausted after about 5 days of use. The metal was stress-relieved as well as in Example I and the surface was acceptably cleaned, but not quite as clean as in Example I.

#### Example III

Metal was first stress-relieved and then cleaned in the same bath compositions and under the same operating conditions as described in Example I, except that in the stress-relieving bath containing 2500 lbs. of fused salt, high temperature steam at about 1200° F. was continuously bubbled into the bottom of the fused bath at the rate of approximately 5 lbs. of steam per hour. It was found after an operating period of 2 weeks that there were no signs of corrosion on the stress-relieving bath apparatus.

#### Example IV

The same cleaning bath as described in Example I was used in combination with a stress-relieving bath having the composition of 80% sodium hydroxide, 10% sodium chloride, 4% sodium fluoride, 1% sodium aluminate and 5% barium hydroxide octahydrate. It was found that the metal was cleaned equally well as in Example I, there being no apparent deteriorating effect upon the electrolytic cleaning bath by barium hydroxide transferred from the stress-relieving bath. It was further found that there were no signs of corrosion upon the stress-relieving apparatus until about 12 days of use of this bath, thereby indicating that the hydrated barium salt has a substantial effect to inhibit corrosion which is substantially superior to that of borax.

As thus described, stress-relieving of metals as a primary step applied prior to cleaning of the metal is desirably effected in a bath having either the same salt composition as that of the electrolytic bath or one having hydrated components of the same composition as the electrolytic bath or having hydrated components of alkali earth metal salts whose anions correspond to those already present in the electrolytic cleaning bath.

Such compositions are outstandingly useful for stress-relieving where the metal is subsequently to be electrolytically cleaned in a molten salt bath, because the stress-relieved metal may be directly transferred from the stress-relieving bath to the electrolytic cleaning bath without contaminating and deteriorating the electrolytic cleaning bath as to interfere with its electrolytic cleaning function. Moreover, without electrolysis, such components as described in the stress-relieving bath, do not adversely affect oxides and scale upon the metal to be stress-relieved whereby the metal is subsequently efficiently cleaned in an electrolytic cleaning bath of the molten salt type.

Moreover, in another aspect of this invention, it is found that if the electrolytic bath is humidified by passing therein continuously or intermittently small quantities of water vapor, substantial corrosion of the stress-relieving apparatus may be inhibited. That same humidification may be effected by using, in the stress-relieving bath, salts normally useful in the electrolytic cleaning bath, one or more of which are desirably in the hydrated form to contain water of crystallization. Where an hydrated salt is used to supply water other than a hydrated salt of the type used in the electrolytic cleaning bath for humidification of the stress-relieving bath, that salt may be an alkali earth metal salt having an anion corresponding to those present in the electrolytic cleaning bath, preferably a hydrated hydroxide of an alkali earth metal, and barium hydroxide of this group, is outstanding for this purpose.

We claim:

1. The method of cleaning and stress-relieving ferrous metal having adherent surface impurities of the character of oxides and scale comprising first heat treating the metal in a non-electrolytic stress-relieving bath at a temperature of about 1100 to 1350° F., and then transferring the stress-relieved metal coated with salts of the stress-relieving bath to an electrolytic cleaning bath of the molten salt type maintained at a temperature in the range of about 600 to 1000° F. and cleaning the metal therein electrolytically, the molten salt composition of both baths comprising about 75 to 90% of caustic alkali, up to about

15% of sodium chloride, up to about 6% of alkali metal fluoride, up to about 10% alkali metal cyanide, 0 to 10% alkali metal silicate and the remainder, at least 0.5%, selected from the group consisting of sodium aluminate and alkali metal borate.

5. The method as defined in claim 1, wherein the molten salt stress-relieving bath is humidified by addition of water vapor thereto.

10. The method as defined in claim 1, wherein the molten salt stress-relieving bath is humidified by having one of its salt components in hydrated form.

15. The method as defined in claim 1, wherein the molten salt stress-relieving bath has added thereto 1 to 15% of a hydrated alkali earth metal hydroxide.

15. The method as defined in claim 1, wherein the molten salt stress-relieving bath has added thereto 1 to 15% of hydrated barium hydroxide.

20. A stress-relieving bath composition in which the metal parts are heated for stress-relieving, comprising by weight, about 75 to 90% sodium hydroxide, 7 to 13% sodium chloride, up to about 6% sodium fluoride, 0.5 to 5% sodium aluminate and 1 to 15% of a hydrated hydroxide of an alkali earth metal.

25. A stress-relieving molten salt bath composition in which metal parts are heated for stress-relieving comprising about 75 to 90% sodium hydroxide, 7 to 15% sodium chloride, up to about 6% sodium fluoride, 0.5 to 5% sodium aluminate and 1 to 15% hydrated barium hydroxide.

30. A stress relieving molten salt bath composition in which metal parts are heated for stress relieving, comprising about 75 to 90% sodium hydroxide, 7 to 15% sodium chloride, 0.5 to 5% sodium aluminate and 1 to 15% of hydrated barium hydroxide.

35. References Cited in the file of this patent

UNITED STATES PATENTS

|           |         |       |               |
|-----------|---------|-------|---------------|
| 2,458,663 | Webster | ----- | Jan. 11, 1949 |
| 2,468,006 | Webster | ----- | Apr. 19, 1949 |
| 2,738,294 | Spence  | ----- | Mar. 13, 1956 |